

## UNITED STATES PATENT OFFICE

1,956,327

## MATERIAL FOR ARC WELDING

Theophil E. Jerabek, East Cleveland, Ohio, assignor to The Lincoln Electric Company, Cleveland, Ohio, a corporation of Ohio

No Drawing. Application February 8, 1932,  
Serial No. 591,757

7 Claims. (Cl. 219—8)

This invention relates as indicated to materials for arc welding, and has specific reference to the employment of certain materials for the purpose of providing a protective coating over 5 the pool of molten metal formed upon or in the work by the presentation thereto in arcing relation of a suitable electrode.

It has been well known in the art of electric arc welding that the pool of molten metal formed 10 in the vicinity of the arc area should be protected by a suitable coating or blanket of fluxing material effective to exclude the atmosphere from the metal. Numerous materials such as clay have been employed as a coating on the weld rod for 15 supplying this protective covering for the pool of molten metal.

All materials which have been employed for the above defined purpose have undesirable characteristics of which those presently to be enumerated 20 are notable examples.

A prominent characteristic of the coating on the pool of molten metal supplied by materials heretofore employed is that such coating usually breaks up into globules or like particles which 25 float upon the pool of molten metal similar to pieces of wood or like material floating on a body of water.

This segregation of the protective material is objectionable from two main standpoints. When 30 the coating segregates in the above defined manner, the intermediate areas of the surface of the pool of molten metal will be unprotected from the atmosphere and to this extent the flux layer fails to serve the function for which the same is 35 employed. The second objectionable feature is that, due to the separation of this coating into segregated islands, each separate globule or island will leave an indentation in the surface of metal after the same has cooled and each indentation 40 will be commensurate with the mass and area of such island similarly as a floating block of wood leaves an impression in the ice as the water is frozen.

Materials of the character heretofore employed 45 having the above named undesirable characteristics have had a tendency, due to their separation into floating islands, to collect in ridges along the sides of the seam thereby producing what is commonly termed "under-cutting" along the sides 50 of the weld metal.

In order that any fluxing material designed to float upon the pool of molten metal shall not form 55 objectionable depressions therein, it is essential that such coating be either of a relatively low specific gravity or porous and fluffy to the ex-

tent that it will readily come to the surface of the pool of molten metal and freely float thereon during solidification of the metal.

After the weld metal has solidified, the flux coating should be readily and completely removable, so that if an additional layer of weld metal is to be deposited, there will be no flux inclusions in the resultant metal deposit.

It is among the objects of my invention to provide materials adapted to form a protective flux covering over the pool of the molten metal which shall have none of the above-named undesirable characteristics, but which shall be distributed over the pool of metal in a uniform film and which shall be capable of being quickly and easily removed without the occurrence thereunder of objectionable under-cuts. Other objects of my invention will appear as the description proceeds.

To the accomplishment of the foregoing and related ends, said invention, then consists of the 75 steps hereinafter fully described and particularly pointed out in the claims, the following description setting forth in detail certain steps embodying the invention, such disclosed steps constituting, however, but one of the various ways in which 80 the principle of the invention may be used.

Among the materials which I have found to be best suited to the above described purposes is titanium dioxide, which may be supplied to the pool of molten metal as a layer or coating on 85 the fusible electrode presented in arcing relation to the work. The titanium dioxide may be bound and secured to the surface of the weld rod by a suitable binder such as sodium silicate.

If titanium dioxide is employed merely in 90 combination with sodium silicate as a binder, it is noted that the flux covering over the pool of molten metal floats as a uniform film which is not broken up into separate islands or globules. Accordingly, there are no local areas of depression in the metal as the same cools and, hence, when the film resulting from the use of titanium dioxide is removed, the surface of the weld metal is very uniform and free from all under-cutting.

The use of titanium dioxide alone with a suitable binder, such as sodium silicate, is, for certain reasons, undesirable, however, due to the fact that the resultant coating on the weld metal adheres so tenaciously thereto that it is very difficult to remove after the metal has solidified.

I have found that a coating which is very light and friable and which can be readily and completely removed after the weld metal has solidified may be produced by employing certain substances in combination with titanium dioxide.

The substances which I have discovered produce the desired results are broadly classified as iron-containing silicates and magnesium containing silicates.

5 Chemically pure magnesium silicate produces the desired results but it may be found more practicable to employ asbestos. Other substances which I have tried and found to produce successful results are talc,  $H_2Mg_3(SiO_3)_4$ ; 10 chrysotile,  $H_4Mg_3Si_2O_9$ ; amosite  $FeSiO_3$ ; crocidolite,  $NaFe(SiO_3)_2FeSiO_3$ ; anthophyllite,  $Fe(Mg)SiO_3$ ; tremolite,  $CaMg_3(SiO_3)_4$ ; actinolite,  $Ca(Mg,Fe)_3(SiO_3)_4$ . The combination of titanium dioxide with a 15 magnesium-containing silicate or an iron containing silicate or both produces a resultant slag coating over the weld metal which extends uniformly over the entire area of the metal, thereby affording complete protection of the metal from 20 the atmosphere. This desirable characteristic of the resultant covering may be due to a number of reasons, such as the melting point of this resultant slag, the viscosity of such slag, the surface tension of such slag, which is so low that there 25 is no segregation into islands, and the fact that the specific gravity of the slag is lower than that of the molten metal. The slag resulting from the above defined coating may likewise have an effect on the surface tension and fluidity of 30 the molten metal, all of which cooperate in producing the desirable results.

When a slag coating is formed on the molten metal in the above defined manner, it will be noted that such coating extends uniformly over 35 the pool while the metal is in its molten state and, due to the uniformity of such film or layer, there will be no local areas in which depressions occur in the metal after the same solidifies. The coating formed in this manner is extremely friable, readily coalescent, very light, and can be 40 very readily removed from the weld metal.

Other modes of applying the principle of my invention may be employed instead of the one

explained, change being made as regards the composition and method herein disclosed, provided the ingredients or steps stated by any of the following claims or the equivalent of such stated ingredients or steps be employed.

80

I, therefore, particularly point out and distinctly claim as my invention:

1. A covered weld-rod for arc welding comprising a metallic rod provided with an adherent covering including titanium dioxide and a magnesium-containing silicate. 85

2. A covered weld-rod for arc welding comprising a metallic rod provided with an adherent covering including titanium dioxide and asbestos. 90

3. A covered weld-rod for arc welding comprising a metallic rod provided with an adherent covering including titanium dioxide and an iron-containing silicate. 95

4. A covered weld-rod for arc welding comprising a metallic rod provided with an adherent covering including titanium dioxide and at least one substance of the group containing iron-containing silicates and magnesium-containing silicates. 100

5. A covered weld-rod for arc welding comprising a metallic rod provided with an adherent covering including titanium dioxide and at least one substance of the group containing magnesium silicate, iron silicate, asbestos, talc, chrysotile, amosite, crocidolite, anthophyllite, tremolite, and 105 actinolite.

6. A covered weldrod for arc welding comprising a metallic rod provided with an adherent covering including a substance containing titanium dioxide, and at least one substance of the 110 group containing iron-containing silicates and magnesium-containing silicates.

7. A slag-forming composition for use in electric arc welding comprising in combination a substance containing titanium dioxide, and at least one substance of the group containing iron-containing silicates and magnesium-containing silicates. 115

THEOPHIL E. JERABEK.

120

## DISCLAIMER

1,956,327.—*Theophil E. Jerabek*, East Cleveland, Ohio. MATERIAL FOR ARC WELDING. Patent dated April 24, 1934. Disclaimer filed January 19, 1940, by the assignee, *The Lincoln Electric Company*.

Hereby enters this disclaimer to the claims in said specification as follows—

In each of claims 1, 2, 3, 4, and 5, we disclaim any covering set forth in said claims, respectively, which includes, in addition to the constituents named, any substantial amount of a halogen-containing compound.

In claim 6 we disclaim any covering set forth in said claim, which includes, in addition to the constituents named, any substantial amount of a nonsilicious slag-forming constituent.

In claim 7 we disclaim any composition set forth in said claim which includes, in addition to the constituents named, any substantial amount of a halogen-containing compound.

[*Official Gazette February 13, 1940.*]

The substances which I have discovered produce the desired results are broadly classified as iron-containing silicates and magnesium containing silicates.

5 Chemically pure magnesium silicate produces the desired results but it may be found more practicable to employ asbestos. Other substances which I have tried and found to produce successful results are talc,  $H_2Mg_3(SiO_3)_4$ ; 10 chrysotile,  $H_4Mg_3Si_2O_9$ ; amosite  $FeSiO_3$ ; crocidolite,  $NaFe(SiO_3)_2FeSiO_3$ ; anthophyllite,  $Fe(Mg)SiO_3$ ; tremolite,  $CaMg_3(SiO_3)_4$ ; actinolite,  $Ca(Mg,Fe)_3(SiO_3)_4$ .

The combination of titanium dioxide with a 15 magnesium-containing silicate or an iron containing silicate or both produces a resultant slag coating over the weld metal which extends uniformly over the entire area of the metal, thereby affording complete protection of the metal from 20 the atmosphere. This desirable characteristic of the resultant covering may be due to a number of reasons, such as the melting point of this resultant slag, the viscosity of such slag, the surface tension of such slag, which is so low that there 25 is no segregation into islands, and the fact that the specific gravity of the slag is lower than that of the molten metal. The slag resulting from the above defined coating may likewise have an effect on the surface tension and fluidity of 30 the molten metal, all of which cooperate in producing the desirable results.

When a slag coating is formed on the molten metal in the above defined manner, it will be noted that such coating extends uniformly over 35 the pool while the metal is in its molten state and, due to the uniformity of such film or layer, there will be no local areas in which depressions occur in the metal after the same solidifies. The coating formed in this manner is extremely friable, readily coalescent, very light, and can be 40 very readily removed from the weld metal.

Other modes of applying the principle of my invention may be employed instead of the one

explained, change being made as regards the composition and method herein disclosed, provided the ingredients or steps stated by any of the following claims or the equivalent of such stated ingredients or steps be employed.

80

I, therefore, particularly point out and distinctly claim as my invention:

1. A covered weld-rod for arc welding comprising a metallic rod provided with an adherent covering including titanium dioxide and a magnesium-containing silicate.

85

2. A covered weld-rod for arc welding comprising a metallic rod provided with an adherent covering including titanium dioxide and asbestos.

90

3. A covered weld-rod for arc welding comprising a metallic rod provided with an adherent covering including titanium dioxide and an iron-containing silicate.

4. A covered weld-rod for arc welding comprising a metallic rod provided with an adherent covering including titanium dioxide and at least one substance of the group containing iron-containing silicates and magnesium-containing silicates.

95

5. A covered weld-rod for arc welding comprising a metallic rod provided with an adherent covering including titanium dioxide and at least one substance of the group containing magnesium silicate, iron silicate, asbestos, talc, chrysotile, amosite, crocidolite, anthophyllite, tremolite, and actinolite.

100

6. A covered weldrod for arc welding comprising a metallic rod provided with an adherent covering including a substance containing titanium dioxide, and at least one substance of the group containing iron-containing silicates and magnesium-containing silicates.

105

7. A slag-forming composition for use in electric arc welding comprising in combination a substance containing titanium dioxide, and at least one substance of the group containing iron-containing silicates and magnesium-containing silicates.

110

THEOPHIL E. JERABEK.

115

120

## DISCLAIMER

1,956,327.—*Theophil E. Jerabek*, East Cleveland, Ohio. MATERIAL FOR ARC WELDING. Patent dated April 24, 1934. Disclaimer filed January 19, 1940, by the assignee, *The Lincoln Electric Company*.

Hereby enters this disclaimer to the claims in said specification as follows—

In each of claims 1, 2, 3, 4, and 5, we disclaim any covering set forth in said claims, respectively, which includes, in addition to the constituents named, any substantial amount of a halogen-containing compound.

In claim 6 we disclaim any covering set forth in said claim, which includes, in addition to the constituents named, any substantial amount of a nonsilicious slag-forming constituent.

In claim 7 we disclaim any composition set forth in said claim which includes, in addition to the constituents named, any substantial amount of a halogen-containing compound.

[*Official Gazette February 13, 1940.*]